

# United States Patent Office

3,099,132

13

3,999,132

3,097,152

**PROPELLANT METHOD USING ORGANIC THIO-  
PHOSPHITES WITH HYDROGEN PEROXIDE**

PHOSPHITES WITHIN THE  
Paul C. Condit, Berkeley, Calif., assignor to California  
Research Corporation, San Francisco, Calif., a corpo-  
ration of Delaware. 2,641,625

ration of Delaware No. Drawing. Filed June 20, 1952, Ser. No. 294,727

No Drawing. Filed June 25, 1932. Serial No. 620,311  
1 Claim. (Cl. 60—35.4)

This invention relates to self-igniting propellant fuel 10 compositions.

Self-igniting compositions of various kinds have for many years found use in the construction of assorted tools of war for use against personnel and property. More recently, it has been recognized that self-igniting compositions are useful as propellants for rockets, guided missiles, and aircraft powered by jet or thrust engines.

In the development of fuels for rockets, thrust engines, etc., it has been recognized that the property of self-ignition in the propellant fuel, while not absolutely essential, constitutes a major convenience in the construction and operation of these devices. In the development of rocket fuels, two types have been recognized: Monergolic fuels, or monergols, i.e., unitary compositions which require ignition by spark, pyrotechnic charge or otherwise and, once started, they continue to burn on being sprayed into the hot zone; and hypergolic fuels, or hypergols, which comprise two or more components which are separately stored and which spontaneously ignite upon proper mixing in a combustion chamber. The individual components of the hypergolic mixture are not self-igniting.

Monogols so far developed have proved unreliable in that they have all shown a tendency to backfire from the combustion chamber to storage tanks. This difficulty is not encountered with hypergolic fuels since self-ignition occurs only upon mixing of the individual components which are not themselves self-igniting and neither of which alone has the property of undergoing self-sustained combustion after ignition.

Hypergolic propellants may be generally described as mixtures of a reducing component and an oxidizing component. When the two components are mixed, there is a short period during which the mixture exists as a composition of matter. During this short period relatively slow reaction of the two components is apparently initiated and this relatively slow reaction is followed by spontaneous ignition of the fuel. The ignition delay period is quite short, being substantially less than one second and being preferably not more than about fifty milliseconds.

The reducing component of a hypergolic propellant should have certain properties as follows: It should ignite spontaneously upon being combined with the selected oxidizing agent; the ignition delay period should be short, preferably not exceeding 50 milliseconds; it should have a low freezing point so that it can be pumped to the combustion chamber at the low temperatures prevailing at high altitudes; it should have a high boiling point to facilitate handling and increase its safety in use; it should be chemically stable in storage; it should have a relatively low viscosity at low temperatures; it should form gaseous oxidation products and the average molecular weight of these products should be as low as possible in order that the specific impulse (pounds thrust/pounds propellant/second) be high. In addition to the foregoing properties, it is desirable that self-ignition of the mixture of the reducing component and the oxidizing agent be rapid over a wide temperature range; that the reducing component have a high density so that the volume of fuel tanks may be reduced; that the material

be non-toxic and easy to handle; that it have a high heat of combustion; and that it be non-corrosive.

heat of combustion, and that  
5 It has now been found that the foregoing property  
requirements of the reducing component are remarkably  
well satisfied by trialkyl trithiophosphites containing 1  
to 4 carbon atoms in each alkyl group and by trialkenyl  
trithiophosphites containing 2 to 4 carbon atoms in each  
alkenyl group. Mixtures of these trithiophosphites with  
10 an oxidizing agent of the group consisting of concentrated  
nitric acid and concentrated hydrogen peroxide are self-  
igniting over a wide range of temperatures and are char-  
acterized by short ignition delay periods.

The reducing component of these hypergolic propellants may be prepared either by reacting a mercaptan with phosphorous trichloride or by oxidizing a mercaptan to a disulfide and then reacting the disulfide with elemental phosphorous as indicated in the following equations:



R is an alkyl group containing 1 to 4 carbon atoms or an alkenyl group containing 2 to 4 carbon atoms.

The boiling point, melting point and density of some of the trithiophosphites are tabulated below:

| Alkyl Groups  | B.P., ° F. | Press.,<br>mm. Hg | M.P., ° F.        | <i>d</i> <sup>4</sup> |
|---------------|------------|-------------------|-------------------|-----------------------|
| Methyl.....   | 208-210    | 5                 | below -100.....   | 1.1883                |
| Ethyl.....    | 284-289    | 18                | -70.....          | 1.1277                |
| n-Propyl..... | 327-336    | 15                | -85 to -83.....   | 1.0773                |
| n-butyl.....  | 345-356    | 15                | -150 to -148..... |                       |

Trimethyl trithiophosphite, triethyl trithiophosphite, 40 tripropyl trithiophosphites, tributyl trithiophosphites, tri-vinyl trithiophosphite, triallyl trithiophosphite and tri-butyl trithiophosphites are all characterized by high boiling points, low melting points and relatively high densities, and all of them ignite spontaneously and rapidly when mixed with either concentrated nitric acid or concentrated hydrogen peroxide.

The term "concentrated nitric acid" as employed above and in the appended claims is intended to include several readily available nitric acid compositions described hereinafter. Ordinary white fuming nitric acid, i.e., nitric acid having a purity in the range from 95 to 100% by weight  $\text{HNO}_2$ , particularly commercial fuming nitric acid composed of 98.5% by weight of  $\text{HNO}_3$ , and 1.5% by weight of water are satisfactory. A small amount of  $\text{N}_2\text{O}_5$  may desirably be added to commercial fuming nitric acid to render it anhydrous. A nitric acid composition containing 92-98 parts by weight of  $\text{HNO}_3$ , 1 to 4 parts by weight of water, and 1 to 4 parts by weight of sodium nitrite, which is characterized by a very low freezing point and high storage stability, is effective. Red fuming nitric acid, i.e., fuming nitric acid containing 2 to 20% by weight, ordinarily about 7½% by weight of nitrogen dioxide, is effective. Fuming nitric acid containing from 2 to 20% by weight of sulfuric acid is also effective. Ordinarily, from 12 to 15% by weight of sulfuric acid will be employed. Fuming nitric acid containing from 2 to 20% by weight of nitrosyl sulfuric acid is also an effective oxidizing agent. The nitrogen dioxide, sulfuric acid, and nitrosyl sulfuric acid are added to fuming nitric acid as ignition accelerators. While they have the effect of shortening the ignition delay period of the hypergolic fuel mixture, their inclu-

sion in the nitric acid introduces problems of sludging and decomposition on storage. The trithiophosphite reducing components of the hypergolic fuels of this invention are especially attractive in that they ignite very rapidly with white fuming nitric acid and the storage problems which attend the addition of ignition accelerators can be avoided. In addition to the nitric acid compositions above, mixtures of nitric oxide and nitrogen dioxide may be employed as the oxidizing component of the hypergolic fuel. For example, a mixture of 60-80% by weight of  $\text{NO}_2$  and 20-40% by weight of NO is effective.

When hydrogen peroxide is employed as the oxidizing component of the hypergolic fuel, it should be employed at high concentration, above about 75% by weight, and preferably above 90% by weight, the remainder being water.

The following examples illustrate the propellant of this invention:

*Example 1*

1 volume of triethyl trithiophosphite and 3 volumes of nitric acid composed of 92.16 parts by weight of  $\text{HNO}_3$ , 3.84 parts by weight of water, and 4 parts by weight of sodium nitrite were mixed at 75° F. 12 milliseconds after mixing spontaneous ignition of the mixture occurred. The triethyl trithiophosphite was very rapidly oxidized, forming water vapor, carbon dioxide, carbon monoxide, sulfur dioxide and oxides of phosphorus. The acid was reduced forming water vapor, nitrogen and nitrogen oxides. The ignition delay was measured by mixing the triethyl trithiophosphite and the acid in an especially constructed oxidizer cylinder so arranged that at the instant of mixing the trithiophosphite and the acid, an electrode was grounded initiating a pulse to an electronic timer to commence the measurement of the delay. Soon after the acid contacted the trithiophosphite, ignition occurred. Ionization caused by the flame grounded a tubular electrode to the walls of the oxidizer cylinder, furnishing the terminating pulse to the electronic timer to complete the delay measurement. Ignition delays as measured by this device are accurate within one millisecond.

Ignition delays of triethyl trithiophosphite and the acid above described were made at several temperatures and the following results were obtained: At 20° F. the ignition delay was 10 milliseconds; at -40° F. the ignition delay was 8 milliseconds; at -70° F. the ignition delay was 10.5 milliseconds; at -80° F. the ignition delay was 37 milliseconds; and at -90° F. the ignition delay was 55 milliseconds.

*Example 2*

One volume of trissecondarybutyl trithiophosphite was mixed with 3 volumes of white fuming nitric acid containing 98.5% of  $\text{HNO}_3$  and 1.5% of water at -40° F. The ignition delay, measured as in Example 1, was 49 milliseconds. Trissecondarybutyl trithiophosphite is a very viscous liquid at -40° F. and a part of the length of the ignition delay may be attributed to poor mixing with the nitric acid.

*Example 3*

One volume of triallyl trithiophosphite was mixed with 3 volumes of commercial fuming nitric acid at -40° F. The ignition delay, measured as in Example 1, was 49 milliseconds. Triallyl trithiophosphite is very viscous at low temperatures and a part of this delay may be attributed to poor mixing with the nitric acid.

*Example 4*

Ignition delay periods were measured at several temperatures for mixtures of 1 volume of trimethyl trithiophosphite with 3 volumes of white fuming nitric acid containing 4% by weight of sodium nitrite. The following results were obtained: At 75° F. the ignition delay was 6 milliseconds; at 20° F. the ignition delay was 3

milliseconds; at -40° F. the ignition delay was 4.5 milliseconds; at -70° F. the ignition delay was 6 milliseconds; at -80° F. the ignition delay was 19.5 milliseconds; and at -90° F. the ignition delay was 71 milliseconds.

*Example 5*

One volume of trimethyl trithiophosphite and 3 volumes of 80% hydrogen peroxide were mixed. The ignition delay period was not measured, but visual observation indicated that the delay period was short, the materials appearing to burst into flame immediately upon mixing.

*Example 6*

A mixture of trivinyl trithiophosphite and white fuming nitric acid ignites immediately upon mixing.

*Example 7*

A mixture of tributenyl trithiophosphite and white fuming nitric acid ignites immediately upon mixing.

In the foregoing examples the trithiophosphites of the invention are shown to ignite spontaneously when mixed with white fuming nitric acid which is the least active of the nitric acids above described. Red fuming nitric acid, i.e., nitric acid containing dissolved  $\text{NO}_2$ , mixed acid, i.e., nitric acid containing 12-15%  $\text{H}_2\text{SO}_4$ , nitric acid containing nitrosyl sulfuric acid and the mixed oxides of nitrogen all give ignition delay periods with the trithiophosphites which are as short or shorter than those obtained with white fuming nitric acid in the examples.

In employing the hypergolic fuel compositions of the invention to operate a thrust or rocket engine, the oxidizing component and the trithiophosphite component are stored in separate tanks connected by lines to the combustion chamber of the engine. The two components are pumped through the lines to the combustion chambers in appropriate amounts. Ordinarily, the weight of oxidizing agent pumped to the combustion chamber is from 2 to 4 times the weight of the trithiophosphite. Highest specific impulses are observed when the quantity of oxidizing agent is slightly less than the amount stoichiometrically required for the complex oxidation of the trithiophosphite component.

The capacity of the trialkyl trithiophosphites to ignite spontaneously upon mixing with the described oxidizing agents is so great that these materials may be mixed with other reducing agents which exhibit longer ignition delay periods, or with materials such as light hydrocarbon oils which do not ignite spontaneously, to produce blends exhibiting ignition delay periods below 50 milliseconds at temperatures about -40° F. and higher.

I claim:

55 A rocket propulsion method, which method comprises injecting separately and simultaneously into the combustion chamber of a rocket motor a fuel consisting of a trialkyl trithiophosphite selected from the group consisting of trialkyl trithiophosphites containing from 1 to 4 carbon atoms in each alkyl group and a tri- lower alkenyl trithiophosphite 60 and an oxidizing agent consisting of concentrated hydrogen peroxide, in an amount and at a rate sufficient to initiate a hypergolic reaction with and to support combustion of the fuel.

References Cited in the file of this patent

UNITED STATES PATENTS

|           |                 |               |
|-----------|-----------------|---------------|
| 2,261,227 | Cloud           | Nov. 4, 1941  |
| 2,382,905 | Pedersen et al. | Aug. 14, 1945 |
| 2,542,370 | Stevens et al.  | Feb. 20, 1951 |
| 2,573,471 | Malina et al.   | Oct. 30, 1951 |

OTHER REFERENCES

Journal of the American Rocket Society, No. 72, December 1947, pages 17, 33, and 35. Copy in Scientific Library.